

Feb. 11, 1930.

L. P. SCHWEITZER

1,746,366

INSULATING LAYERS FOR ELECTRICAL CONDENSERS

Filed Oct. 24, 1928

*Fig. 1*



*Fig. 2*



*Fig. 3*



*Fig. 4*



INVENTOR  
Louis P. Schweitzer  
BY  
Oscarick Breitenfeld  
ATTORNEY

## UNITED STATES PATENT OFFICE

LOUIS P. SCHWEITZER, OF NEW YORK, N. Y.

## INSULATING LAYERS FOR ELECTRICAL CONDENSERS

Application filed October 24, 1928. Serial No. 314,637.

My present invention relates generally to electrical condensers, and has particular reference to the insulating layers of so-called paper-dielectric condensers.

In the manufacture of condensers of the foregoing general character, layers of conducting and non-conducting material, usually foil and paper, are interwound in alternate relationship, the condenser body thus formed is then subjected to heat and vacuum treatment to expel all entrained moisture and air, and it is then impregnated with a suitable dielectric material, such as wax. The length of life of such condensers, and the voltage which they are enabled to withstand, are dependent to a large extent upon the thoroughness of such impregnation. Since breakdown has been found to result from the passage of leakage currents through the impregnated insulating layers, it is most important to provide such layers of a character which will most thoroughly withstand and prevent the passage of such currents.

My invention relates in general to an improvement in the provision of such insulating layers and resides from one aspect in a method of enhancing the thoroughness with which such layers are treated to render them impervious to the passage of leakage currents. From another aspect, my invention resides in the provision of an improved insulating layer to be used in the manufacture of such condensers.

One feature of my invention resides in employing an auxiliary dielectric material which will supplement the desired effect of the usual impregnating medium, such as wax. More particularly, it is a feature of my invention to provide an insulating strip of paper with an initial coating which will render such coated paper particularly valuable for employment thereafter in the usual manner.

Thus, from a third aspect, my invention relates to paper manufacture, it being one object of my invention to provide a paper having certain improved qualities which render it particularly adaptable for the manufacture of paper-dielectric condensers.

Being mindful of the general steps of condenser manufacture, as outlined above, and

seeking to avoid any alteration of such steps, I have provided a paper insulating layer which has been treated in a particular manner with an auxiliary dielectric material but which is still susceptible to impregnation in the usual manner by the usual wax dielectric material. In accordance with my invention, I start with a porous strip of paper and coat the same on one surface only with an extremely thin and intimately associated continuous layer of unporous dielectric material. I have found pyroxylin to be peculiarly adapted to the contemplated purposes.

Since pyroxylin is an excellent insulating medium, I have found that by providing an extremely fine yet continuous and impervious coating thereof upon one surface of a porous paper strip, such strip is enhanced for insulating purposes by virtue of an initially provided impervious insulating wall. At the same time, the paper is susceptible to impregnation in the usual manner during the regular course of condenser manufacture.

I have found that the carrying out of my invention results in more than the provision of two superposed and separable layers of paper and pyroxylin. Since the latter is peculiarly capable of application in liquid form, although it dries with great rapidity, it has certain impregnating characteristics which cause the coating to form portions which extend into the interior of the paper through certain pores of the latter and toward the uncoated surface thereof. In this way, an extremely intimate association results, producing a treated paper of a novel character and having qualities of particular value for employment as an insulating layer.

For the attainment of the foregoing objects and such other objects as may herein-after appear or be pointed out, my invention may be carried out as illustrated in the accompanying drawings, in which—

Figure 1 is a cross-sectional view on an enlarged scale of an untreated paper strip;

Figure 2 is a diagrammatic representation of the treatment to which such strip is subjected;

Figure 3 is a cross-sectional view similar

to Figure 1 showing the effect of such treatment;

Figure 3A is a perspective view of a completely wound and compressed condenser body of the character in which the present insulating layer is employed; and

Figure 4 is a fragmentary cross-sectional view through a completed electrical condenser embodying the improved insulating layer.

The strip of paper 10 shown in Figure 1 may be of the usual variety generally employed for purposes of condenser manufacture, being of predetermined uniform thickness and grade. It is usually unsized and of substantially uniform porous consistency.

By means of any suitable apparatus, I wind such strip from a roll 11 to a roll 12, and during the passage from one to the other 20 I pass the strip over a roller 13 having its lower portion immersed in a bath 14 of the auxiliary insulating material desired. Where such bath comprises liquid pyroxylin, I am enabled to provide an extremely thin yet 25 continuous and impervious coating of the pyroxylin upon the strip 10 in a comparatively simple and inexpensive manner. Since the pyroxylin dries very quickly, I may allow the same to dry merely during its passage from 30 the bath to the roll 12, or I may provide suitable heating means or the like for facilitating such drying.

In Figure 3 I have shown the resultant improved and treated paper strip. A continuous and unporous coating 15 of pyroxylin presents an exceptionally smooth and unbroken surface 16 on one side of the strip. The other side 17 of the strip still presents the same porous surface as it did before. The 40 coating 15 will be found to have portions 18 extending into the interior of the paper through certain pores of the latter and toward the uncoated surface 17. Thus, it will be seen that my treatment, though resembling 45 impregnation to a certain extent and resembling pure coating to a certain extent is, as a matter of fact, a combination of the two, the resultant strip being a unitary article having the novel and improved characteristics hereinbefore referred to.

This improved unitary strip may be supplied in rolls in the usual manner to the manufacturers of condensers. It may then be interwound in the usual manner with strips 55 of conducting material such as foil, and the condenser bodies may be subjected to the heat and vacuum treatment and the customary impregnation.

A condenser body of the foregoing character is shown in Figure 3A. One end portion 20 comprises superposed edges of one foil strip (for example, the upper strip 19 of Figure 4), and the opposite end portion 21 comprises superposed edges of the other foil strip (for example, the lower strip 19 of Fig-

ure 4). These end portions are completely insulated from each other by the interwound insulating layer or layers and are therefore usable as terminals in the completed condenser. Usually, a pair of contact terminals or strips 22 and 23 are made to project outwardly from the end portions 20 and 21. In Figure 3A, I have also shown a sticker or label 24 applied to the free ends of the insulating layers or strips to hold the condenser body in wound condition.

A fragmentary cross-section on a greatly enlarged scale through a portion of the completed condenser is shown in Figure 4. The layers 19 are foil sandwiching my improved insulating layer between them, the surface 16 being in close contact with one of the foil strips, and the surface 17 being in close contact with the other foil strip. The usual impregnating medium will have found its way 80 into the paper in the usual manner and will be supplemented by the impervious and non-conducting wall 15. As a result, the completed condenser will have improved qualities 85 imparting increased life and improved capability of withstanding high voltages. Leakage currents may find their way through certain portions of the wax but will find it comparatively difficult to pass completely 90 through the insulating layer by virtue of the obstruction presented by the wall 15.

It will be obvious that changes in the details herein described and illustrated for the purpose of explaining the nature of my invention may be made by those skilled in the 100 art without departing from the spirit and scope of the invention as expressed in the appended claims. It is therefore intended that these details be interpreted as illustrative, and not in a limiting sense.

Having thus described my invention and illustrated its use, what I claim as new and desire to secure by Letters Patent is—

1. In a wound condenser body comprising alternate layers of conducting and non-conducting material, an insulating layer comprising a strip of paper susceptible to impregnation by a dielectric liquid medium, and a continuous and impervious coating of pyroxylin intimately associated with only one 115 surface of said strip.

2. In a wound condenser body comprising alternate layers of conducting and non-conducting material, an insulating layer comprising a strip of paper susceptible to impregnation by a dielectric liquid medium, and a continuous and impervious coating of pyroxyline intimately associated with only one surface of said strip, said coating of pyroxylin having portions which extend into the interior of the paper through certain pores of the latter and toward the opposite uncoated surface.

3. In an electrical condenser comprising interwound alternate layers of conducting and

non-conducting material, an insulating layer comprising a strip of porous paper and a continuous unporous coating of dielectric material intimately associated with one surface thereof, and a second dielectric material in intimate impregnatory association with the entire insulating layer.

4. In an electrical condenser comprising interwound alternate layers of conducting and non-conducting material, an insulating layer comprising a strip of porous paper and a continuous coating of pyroxylin intimately associated with one surface thereof, and a second dielectric material in intimate impregnatory association with the entire insulating layer.

5. In an electrical condenser comprising interwound alternate layers of conducting and non-conducting material, an insulating layer comprising a strip of porous paper and a continuous coating of pyroxylin intimately associated with one surface thereof, and a wax dielectric material in intimate impregnatory association with the entire insulating layer.

25 6. In an electrical condenser comprising interwound alternate layers of conducting and non-conducting material, an insulating layer comprising a strip of porous paper and a continuous unporous coating of dielectric material intimately associated with one surface thereof and having portions which extend through certain pores of the paper toward the uncoated surface of the latter, and a second dielectric material in intimate impregnatory association with the entire insulating layer and filling in the remaining pores.

7. In an electrical condenser comprising interwound alternate layers of conducting and non-conducting material, an insulating layer comprising a strip of porous paper and a continuous coating of pyroxylin intimately associated with one surface thereof and having portions which extend through certain pores of the paper toward the uncoated surface of the latter, and a wax dielectric impregnating material extending from said uncoated surface into the interior of the paper and filling in the remaining pores.

50 In witness whereof I have signed and sealed this specification this 16th day of October, 1928.

LOUIS P. SCHWEITZER.